

## 1

2,911,369

**HIGH TEMPERATURE GREASE CONTAINING FREE METAL BASE AND SILICONE POLYMER OIL**

Stephen J. Zajac, Whiting, and Reuben A. Swenson, Hammond, Ind., assignors to Standard Oil Company, Chicago, Ill., a corporation of Indiana

No Drawing. Application December 28, 1956  
Serial No. 631,072

11 Claims. (Cl. 252—40)

This invention relates to high temperature greases and more particularly pertains to alkali metal and alkaline earth metal soap greases having high temperature stability characteristics and to the method of preparing such greases.

It is an object of the present invention to provide a lubricating grease which is stable at high temperatures with respect to consistency and which is resistant to leakage at high temperatures. Another object of the invention is to provide metal soap greases having high dropping points. Still another object of the invention is to provide lubricating greases which will effectively lubricate bearings operating at high temperatures and which will not melt and/or lose consistency at such operating temperatures. Other objects and advantages of the invention will become apparent from the following description thereof.

U.S. Patent No. 2,684,944, issued July 27, 1954, to S. J. Zajac covers lithium polyorgano siloxane polymer greases containing 10% to 50% of a free basic compound, based on the lithium soap content of the grease, which greases have high temperature stability characteristics. We have now found that the above objects can be attained with a lubricating grease comprising a major proportion of a lubricating oil, from about 0.5% to about 10% of a normally liquid silicone polymer oil, 1% to about 20%, and preferably from about 2% to about 10% of a metal soap of a high molecular weight fatty acid, and a free basic compound in amounts of from about 3.0% to about 500%, and preferably from about 5.0% to about 200%, based on the soap content of the grease.

The metal soaps employed in the grease compositions of the present invention are preferably the alkali metal and the alkaline earth soaps of unsaturated, partially unsaturated or saturated fatty acids or hydroxy fatty acids having at least 12 carbon atoms, and preferably from about 12 to 22 or more carbon atoms. Examples of suitable fatty acids are lauric acid, myristic acid, palmitic acid, stearic acid, behenic acid, oleic acid, hydrogenated fish oil fatty acids, hydrogenated castor oil, hydroxy stearic acid, e.g., 12-hydroxy stearic acid, and the like. The term "high molecular weight fatty acid," as used herein and in the appended claims, means a fatty acid having at least 12 carbon atoms. Examples of suitable metal soaps are lithium stearate, lithium 12-hydroxy stearate, sodium stearate, barium stearate, strontium soap of hydrogenated fish oil fatty acids, barium 12-hydroxy stearate, etc. Mixtures of such soap can also be used.

The specific effectiveness of the various fatty acids varies to some extent, the metal soaps of all of them, however, being effective to various degrees. It is, therefore, not to be implied that the metal soaps of all of the herein-described fatty acids are equivalents.

The required excess alkalinity of the grease is supplied by incorporating in the grease composition from about

## 2

3% to about 500%, or more, and preferably from about 5% to about 200% based on the soap content of the grease, of a basic compound such as basic alkali metal compounds, basic alkaline earth compounds, and high boiling basic organic nitrogen compounds, such as aliphatic or aromatic amines boiling above about 250° F. Examples of suitable basic compounds are sodium hydroxide, potassium hydroxide, lithium hydroxide, lithium oxide, barium hydroxide, barium oxide, calcium hydroxide, calcium oxide, triphenyl amine, octylamine, etc.

The silicone oil polymer employed is suitably a polymeric liquid compound having the general formula



in which R<sub>1</sub>, R<sub>2</sub>, R<sub>3</sub>, R<sub>4</sub>, and R<sub>5</sub> are the same or different hydrocarbon radicals, such as alkyl, aryl, alkaryl or aralkyl radicals and n is an integer greater than 1. Depending upon the extent of condensation or polymerization, the polymer products vary from relatively light liquids to solid resins. However, for the purpose of the present invention, polymers which are high boiling liquids within the lubricating oil viscosity range are preferred. Commercially available compounds of this type are polymers of dimethyl silicone, diethyl silicone, ethylmethyl silicone, diphenyl silicone, ditolyl silicone, methyl phenyl silicone, ethyl phenyl silicone, and the like. Other silicone polymers produced from high molecular weight hydrocarbon groups, such as butyl, amyl, hexyl and above, when economically available can also be used. Compounds of the type above described and the methods of preparing the same are described in U.S. 2,352,974, 2,258,222, 2,371,068 and others. Polymeric organic silicon compounds of this type are also referred to as polymeric dihydrocarbon siloxanes or polyorgano siloxanes.

The lubricating oil vehicle used in the grease can be a mineral oil in the lubricating oil viscosity range, i.e. from about 50 S.S.U. at 100° F. to about 300 S.S.U. at 210° F., or a synthetic hydrocarbon oil such as is obtained by the polymerization of unsaturated hydrocarbons. Other oleaginous materials within the lubricating oil range can be used, such as, for example high molecular weight polyoxalkylene compounds such as polyoxalkylene glycol and esters thereof; aliphatic diesters of dicarboxylic acids such as the butyl, hexyl, ethyl hexyl, decyl, lauryl, etc. esters of sebacic acid, adipic acid, azelaic acid, etc.; polyfluoro derivatives of organic compounds, particularly hydrocarbons, such as trifluorovinyl chloride polymer, trifluorochloroethylene polymer, etc.

Greases of the present invention are easily prepared and do not require the use of solvents. In preparing greases of the present invention, all of the metal soap or soap constituents, all of the polyorgano siloxane, all of the basic compound, preferably in the form of an aqueous solution or suspension and a portion of the oleaginous vehicle are mixed together, slowly heated to a temperature of about 212° F., and maintained at this temperature until the mixture is substantially free of water. When the mixture is substantially anhydrous, and foaming, if any, subsides, the remaining portion of the oleaginous vehicle is added, the batch heated to a temperature of from about 450° F. to about 550° F., and preferably to a temperature of about 500° F. to 510° F., and maintained at said temperature until the reaction is completed. The grease is then filled and cooled. The cooled product, if desired, can be homogenized by well known means.

The grease compositions of the present invention are illustrated by the examples in the following table:

TABLE I

| Component                                   | Examples |        |           |       |           |       |       |
|---------------------------------------------|----------|--------|-----------|-------|-----------|-------|-------|
|                                             | 1        | 2      | 3         | 4     | 5         | 6     | 7     |
| Lithium 12-hydroxy stearate, percent        | 7.0      | 1.50   | 0.75      | 7.2   | 11.0      | 11.0  | 7.0   |
| Lithium hydroxide monohydrate, percent      | 0.75     | 0.75   | 0.375     |       | 1.0       |       |       |
| Silicone Oil (DC 550), <sup>1</sup> percent | 1.50     | 1.50   | 0.75      |       | 2.5       |       | 1.5   |
| Petroleum Oil, Percent                      | 90.75    |        |           | 92.8  |           |       | 91.5  |
| SSU at 100° F.                              | 813      |        |           | 813   |           |       | 813   |
| Petroleum Polymer Oil, <sup>2</sup> Percent |          | 96.25  | 98.13     |       |           |       |       |
| SSU at 100° F.                              |          | 100    | 100       |       | 85.5      | 89.0  |       |
| Synthetic Oil, <sup>3</sup> Percent         |          |        |           |       | 60        | 60    |       |
| SSU at 100° F.                              |          |        |           |       |           |       |       |
| Penetration at 77° F.:                      |          |        |           |       |           |       |       |
| Unworked                                    | 321      | 347    | Too Soft  | 294   | 187       | 245   | 443   |
| Worked                                      | 320      | 341    | Too Soft  | 281   | 192       | 268   | 445   |
| 100,000 strokes                             | 330      |        | Too Soft  | 303   |           |       | 481   |
| Drop Point, ° F.                            | +450     | +460   |           | 300   | +450      | 348   | 327   |
| Hotplate test at 700° F.                    |          |        | No Change | Melts | No Change | Melts | Melts |
|                                             | Change   | Change |           |       |           |       |       |

<sup>1</sup> DO 550—A silicone polymer oil marketed by Dow-Corning.<sup>2</sup> A polybutene having an average molecular weight of 330.<sup>3</sup> Di-isooctyl azelate.

Example 1 is similar to the grease in Example 4 except for the addition of silicone oil and lithium hydroxide. Although it is one grade softer in consistency, it is much superior in high temperature properties.

Example 2 is a low soap content formulation containing lithium silicone polymer. Although it is a soft grease, it has very good high temperature properties.

Example 3 contains 50% less soap and 50% less silicone polymer than Example 2. Although it is a semi-fluid grease, it has good high temperature properties. When placed on a hot plate at 700° F., it maintains its shape and consistency.

Example 4 included for purpose of comparison is a commercial lithium hydroxide stearate grease commonly known as a lithium multipurpose grease.

Example 5 is a lithium hydroxide stearate grease made in a synthetic oil. It also contains silicone polymer. Comparison with Example 6 shows that the drop point of Example 5 is raised +90° F. by the composition of the present invention.

Example 7 is similar to Example 1, but contains no lithium hydroxide monohydrate. This example demonstrates the necessity for the free basic compound in the formulation.

The application of the present invention to greases other than lithium soap greases is demonstrated by the date in Table II.

TABLE II

| Component                      | Example No. |      |      |      |
|--------------------------------|-------------|------|------|------|
|                                | 1           | 2    | 3    | 4    |
| Sodium Stearate, Percent       | 10.5        | 10.5 |      |      |
| Dry Caustic Soda, Percent      | 0.75        |      | 8.7  | 8.7  |
| Barium Stearate, Percent       |             |      | 1.0  |      |
| Barium Hydroxide, Percent      |             | 1.5  | 1.5  |      |
| Silicone Oil (DC-550), Percent | 87.25       | 89.5 | 88.8 | 91.3 |
| Petroleum Oil, Percent         | 300         | 300  | 540  | 540  |
| SSU at 100° F.                 |             |      |      |      |
| Unworked                       | 232         | 315  | 286  | 399  |
| Worked                         | 236         | 280  | 214  | 373  |
| Drop Point, ° F.               | +465        | 365  | +460 | 341  |

Example 1 is a sodium soap grease made in accordance with the present invention and Example 2 is a conventional sodium soap grease made without the excess free alkali and silicone oil. The improved penetration and drop point properties of Example 1 are clearly shown.

Example 3 is a barium soap grease made by the present invention, while Example 4 is a conventional barium soap grease containing no excess free alkalinity and no

silicone oil. Here again the improvement obtained by the present invention is demonstrated.

The effect of the free basic compound is demonstrated by the data in the following Table III.

TABLE III  
Metal hydroxide requirement

|                                        | 1    | 2        | 3    | 4     | 5    |
|----------------------------------------|------|----------|------|-------|------|
| Lithium 12-hydroxy stearate, Percent   | 7.0  | 7.0      | 6.0  | 7.0   | 6.0  |
| Lithium Hydroxide monohydrate, Percent |      | 0.25     | 0.50 | 0.75  | 1.0  |
| Silicone oil (DC-550), Percent         | 1.5  | 1.5      | 1.5  | 1.5   | 1.5  |
| Petroleum Oil, Percent                 | 91.5 | 91.25    | 92.0 | 90.75 | 91.5 |
| S.S.U. at 100° F.                      | 813  | 813      | 813  | 813   | 813  |
| Penetration:                           |      |          |      |       |      |
| Unworked                               | 443  | 423      | 340  | 321   | 318  |
| Worked                                 | 445  | 426      | 336  | 320   | 309  |
| 100,000 strokes                        | 481  | Too Soft | 349  | 330   | 320  |
| Drop point, ° F.                       | 327  | 343      | 429  | +450  | +455 |

In Table III the only ingredient variable is lithium hydroxide. The silicone oil content is constant at 1.5%.

The high temperature stability and lubricating characteristics of the greases of the present invention are given in Table IV together with comparative data for a conventional lithium soap grease.

TABLE IV

| Component                                                | Example |       |       |
|----------------------------------------------------------|---------|-------|-------|
|                                                          | 1       | 2     | 3     |
| Lithium 12-hydroxy stearate, Percent                     | 8.80    | 7.85  | 7.85  |
| Lithium hydroxide, monohydrate, Percent                  | 1.73    | 1.83  | 1.10  |
| Silicone Oil (DC 550), Percent                           | 1.00    | 1.50  |       |
| Petroleum Oil, Percent                                   | 88.47   | 88.82 | 91.05 |
| SSU at 100° F.                                           | 813     | 813   | 300   |
| Penetration at 77° F.:                                   |         |       |       |
| Unworked                                                 | 314     | 305   | 314   |
| Worked                                                   | 309     | 300   | 308   |
| Drop Point, ° F.                                         | +480    | +480  | 384   |
| 10,000 r.p.m. Bearing Test <sup>1</sup> at 350° F., Hrs. | 128     | 138   | 20    |

<sup>1</sup> ABEO-NLGI—Technical Bulletin No. 5—November 1944. Performance characteristics of lubricating grease in anti-friction bearings at elevated temperatures.

The grease of Example 3 was a conventional so-called multipurpose grease.

The high temperature stability property of the greases made in accordance with the present invention cannot be obtained by mixtures of conventional greases and the high temperature stability greases of my U.S. Patent 2,684,944. This is demonstrated by the data in Table V.

5  
TABLE V

| Sample | Product                                         | Drop Point, °F. |
|--------|-------------------------------------------------|-----------------|
| A      | Conventional lithium 12-hydroxy stearate grease | 385             |
| B      | Lithium silicone oil grease of U.S. 2,684,944   | 600             |
| C      | 90% A+10% B                                     | 386             |
| D      | Anhydrous calcium soap grease                   | 289             |
| E      | 90% D+10% B                                     | 289             |
| F      | Hydrous calcium soap grease                     | 217             |
| G      | 90% F+10% B                                     | 218             |

|                                     |         |
|-------------------------------------|---------|
| Composition of grease "A":          | Percent |
| Hydrogenated fatty acid             | 0.69    |
| Hydrogenated castor oil             | 5.90    |
| Lithium hydroxide, H <sub>2</sub> O | 0.90    |
| Ortholeum 300                       | 0.27    |
| Phenothiazine                       | 0.07    |
| Solvent extracted 40 oil            | 91.17   |
| Composition of grease "B":          |         |
| Lithium hydroxy stearate            | 1.5     |
| Lithium hydroxide, H <sub>2</sub> O | 1.5     |
| DC 550 Silicone Oil                 | 97.0    |
| Composition of grease "D":          |         |
| 12-hydroxy stearic acid             | 7.81    |
| Acetic acid                         | 5.86    |
| Lime                                | .50     |
| Solvent extracted 40 oil            | 85.83   |
| Composition of grease "F":          |         |
| Fatty acids                         | 17.00   |
| Hydrated lime                       | 2.21    |
| Dry caustic soda                    | 0.14    |
| Water                               | 0.65    |
| Petroleum oil                       | 80.00   |

The above data show that the mere mixing of a grease of Patent U.S. 2,684,944 and a conventional petroleum oil grease will not give a product having the high temperature characteristics of the grease product of the herein-described invention.

The greases of the present invention can contain added constituents such as anti-oxidants, oiliness agents, extreme pressure additives, anti-foam agents, etc. without in any way departing from the scope of the invention.

Percentages given herein and in the appended claims are weight percentages unless otherwise specified.

While we have described our invention by reference to specific preferred embodiments thereof, it is not intended that the invention be limited thereto, but includes within its scope such modifications and variations as come within the spirit of the appended claims.

We claim:

1. A lubricating grease composition comprising a major proportion of a lubricating oil selected from the group consisting of a hydrocarbon oil, a diester of a dicar-

## 6

boxylic acid and an aliphatic alcohol, and a high molecular weight polyalkylene glycol from about 0.5 to about 10% of a normally liquid silicone polymer oil in the lubricating oil viscosity range, from about 1% to about 20% of a metal soap of a high molecular weight fatty acid selected from the group consisting of an alkali metal soap, an alkaline earth soap and mixtures thereof, and from about 3% to about 500%, based on the metal soap content of said composition, of a free basic compound selected from the group consisting of an alkali metal hydroxide, an alkali metal oxide, an alkaline earth hydroxide and an alkaline earth oxide.

2. A lubricating grease composition as described in claim 1 in which the metal soap is a lithium soap.

15 3. A lubricating grease composition as described in claim 1 in which the metal soap is lithium 12-hydroxy stearate.

4. A lubricating grease composition as described in claim 1 in which the metal soap is the lithium soap of 20 hydrogenated castor oil.

5. A lubricating grease composition as described in claim 1 in which the metal soap is a sodium soap.

6. A lubricating grease composition as described in claim 1 in which the metal soap is a barium soap.

25 7. A lubricating grease composition as described in claim 1 in which the free basic compound is a lithium hydroxide.

8. A lubricating grease composition as described in claim 1 in which the free basic compound is sodium 30 hydroxide.

9. A lubricating grease composition as described in claim 1 in which the free basic compound is hydrated lime.

10. A lubricating grease composition as described in 35 claim 1 in which the free basic compound is barium hydroxide.

11. A lubricating grease composition comprising a major proportion of a hydrocarbon lubricating oil, from about 0.5% to about 10% of a normally liquid silicone polymer oil in the lubricating oil viscosity range, from about 1% to about 20% lithium 12-hydroxy stearate and from about 3% to about 500%, based on the lithium soap content of said composition, of lithium hydroxide.

## 45 References Cited in the file of this patent

## UNITED STATES PATENTS

|           |          |               |
|-----------|----------|---------------|
| 2,417,428 | McLennan | Mar. 18, 1947 |
| 2,684,944 | Zajac    | July 27, 1954 |
| 2,831,812 | Worth    | Apr. 22, 1958 |

## FOREIGN PATENTS

|         |               |                |
|---------|---------------|----------------|
| 736,921 | Great Britain | Sept. 14, 1955 |
|---------|---------------|----------------|

## OTHER REFERENCES

55 Manufacture and Application of Lubricating Greases, Boner, Reinhold Pub. Corp., N.Y., 1954, p. 488.

UNITED STATES PATENT OFFICE  
CERTIFICATE OF CORRECTION

Patent No. 2,911,369

November 3, 1959

Stephen J. Zajac et al.

It is hereby certified that error appears in the printed specification of the above numbered patent requiring correction and that the said Letters Patent should read as corrected below.

Column 2, line 17, after "which" insert -- R, --; column 3, line 48, for "date" read -- data --.

Signed and sealed this 10th day of May 1960.

(SEAL)

Attest:

KARL H. AXLINE

Attesting Officer

ROBERT C. WATSON  
Commissioner of Patents